

June 24, 1969

H. H. BAUM

3,451,338

THERMOGRAPHIC RECORDING SYSTEM

Filed May 11, 1964

Sheet 1 of 2



FIG. 1a



FIG. 1b



FIG. 1c



FIG. 1d



FIG. 2a



FIG. 2b



PHENOLIC MATERIAL (·)

CHROMOGENIC MATERIAL (X)

INVENTOR  
HENRY H. BAUM

BY *Louis A. Kline*  
*Justin S. Kline*

HIS ATTORNEYS

June 24, 1969

H. H. BAUM

3,451,338

THERMOGRAPHIC RECORDING SYSTEM

Filed May 11, 1964

Sheet 2 of 2



INVENTOR  
HENRY H. BAUM

BY

*Louis A. Kline  
John S. Carpenter*

HIS ATTORNEYS

3,451,338

## THERMOGRAPHIC RECORDING SYSTEM

Henry H. Baum, Dayton, Ohio, assignor to The National Cash Register Company, Dayton, Ohio, a corporation of Maryland

Filed May 11, 1964, Ser. No. 366,524

Int. Cl. B41m 5/18

U.S. Cl. 101—469

12 Claims

## ABSTRACT OF THE DISCLOSURE

There is provided by this invention a thermographic method of data-recording and heat-sensitive record sheets comprising chromogenic benzo-indolinospiropyran material and a di-phenol material capable of producing immediate and lasting color when and where the two co-reactant materials are brought into liquid contact, as in a melt. The two described co-reactant materials may be coated in a polymeric film binder on a single base web in interspersion in a single coat or separately incorporated into successive coats, or alternatively the co-reactants may be coated on separate base web sheets to provide a co-reactive pair of sheets.

This invention relates to temperature-responsive record material, and particularly pertains to sheet material having particles of solid material becoming mobile as a fluid phase in recording processes involving thermographic temperatures with heat applied as radiant energy or conducted energy, the fluid mobile material making contact then or later with proximately-located co-reactant solid particles which also may become mobile as a fluid phase to produce a colored mark, and such mark itself being transferable to an unsensitized sheet either at the time the mark is made, or later.

The solid particles provided have a low vapor pressure at temperatures under 60 degrees centigrade (the maximum of living environment), to prevent loss of material by evaporation at room temperature, and will not react on solid-solid contact unless prolonged contact engenders such, so that, if the co-reactant substances are held separated by being on different sheets, the sheets may be brought into contact just before use in a recording operation to make a record by heat application thereto by radiation which produces a thermographic effect, or by conduction in some cases. If the co-reactants are situated in close proximity on the same sheet for providing storage before use and for providing a self-contained sheet sensitive for making a record copy by itself, or two facing sheets are in prolonged contact before use, the particles are isolated against particle contact by their films of material, which will transmit the mobile reactants at the higher-than-60-degree-centigrade recording temperatures, which may range up to 200 degrees centigrade. Thus, where particles of both reactants are interspersed on a sheet, a thin binder of polymeric film material, just sufficient to physically sheath the particles, is used, to prevent solid-solid contact or low vapor pressure contact and consequent premature coloration. If the particles of reactant are on different sheets, one or the other, or both, may have their solid particles of reactant isolated by a binder film material, or a common insert sheet or coating may be used, to separate the sheets. Where a minimum of binder is used between co-reacting particles on the same sheet, an over-layer of film may be used to prevent smudging by winding pressure or stack-contact pressures during storage or handling.

The fluid mobility produced in the reactants by thermographic temperatures is associated with the liquid or vapor state of the material at the high temperature.

The preferred color-producing reactants are phenols on one hand and certain photochromic benzo-indolinospiropyran compounds on the other hand. The preferred phenols are the di-phenols, and the preferred benzo-indolinospiropyrans have the structure (with additional substitution in at least the 8' position).



15 where R, R', and R'' are lower alkyl or phenyl groups. Most commonly R, R', and R'' are methyl groups and in Table I may be so taken unless some other group is indicated by position number. Useful representative compounds are listed in Table I as follows:

TABLE I

|         | Substituent                        | Melting point, degrees centigrade, of derivative |
|---------|------------------------------------|--------------------------------------------------|
| 25 I    | 8'-methoxy*                        | 123-5                                            |
| II      | 8'-ethoxy                          | 83-5                                             |
| III     | 1-ethyl-8'-methoxy                 | 117-8                                            |
| IV      | 3-ethyl-8'-methoxy                 | 96-8                                             |
| V       | 1-amyl-8'-methoxy*                 | 72-7                                             |
| VI      | 1-phenyl-8'-methoxy#               | 161-4                                            |
| VII     | 3-phenyl-8'-methoxy#               | 105-9                                            |
| VIII    | 5-phenyl-8'-methoxy#               | 167-71                                           |
| IX      | 5-phenyl-8'-ethoxy#                | 119-22                                           |
| X       | 7-phenyl-8'-methoxy#               | 142-5                                            |
| XI      | 7-phenyl-8'-ethoxy#                | 117-21                                           |
| XII     | 5-chloro-8'-methoxy*               | 140-1                                            |
| XIII    | 5-chloro-8'-ethoxy                 | 144-5                                            |
| XIV     | 4,7-dichloro-8'-methoxy            | 90-100                                           |
| XV      | 5,8'-dimethoxy                     | 150-3                                            |
| XVI     | 7,8'-dimethoxy                     |                                                  |
| XVII    | 4,7-dimethoxy-8'-ethoxy            | 118-9                                            |
| XIX     | 4,7-diethoxy-8'-methoxy            | 104-6                                            |
| XX      | 5,7,8'-trimethoxy                  | 121-7                                            |
| XXI     | 5,7-dimethoxy-8'-ethoxy            | 111-3                                            |
| XXII    | 4,7-dimethyl-8'-methoxy            | 142-7                                            |
| XXIII   | 4,7-dimethyl-8'-ethoxy             | 82-4                                             |
| XXIV    | 5-B-hydroxyethyl-8'-methoxy        | 78-85                                            |
| XXV     | 6'-chloro-8'-methoxy*              | 123-125                                          |
| XXVI    | 6'-bromo-8'-methoxy                | 182-184                                          |
| XXVII   | 5',6'-dichloro-8'-ethoxy           | 125-126                                          |
| XXIX    | 1-ethyl-6'-chloro-8'-methoxy       | 95-96                                            |
| XXX     | 1-ethyl-6'-bromo-8'-methoxy        | 149-150                                          |
| XXXI    | 1-butyl-6'-chloro-8'-methoxy       | 83-86                                            |
| XXXII   | 3-propyl-6'-chloro-8'-methoxy      | 121-123                                          |
| XXXIII  | 1-phenyl-8'-ethoxy#                | 134-136                                          |
| XXXIV   | 1-phenyl-3-ethyl-8'-methoxy#       | 111-114                                          |
| XXXV    | 1-phenyl-3-propyl-8'-methoxy#      | 145-147                                          |
| XXXVI   | 1-phenyl-6'-chloro-8'-methoxy#     | 153-155                                          |
| XXXVII  | 1-phenyl-5',6'-dichloro-8'-ethoxy# | 121-122                                          |
| XXXVIII | 3-propyl-3-phenyl-8'-methoxy#      | 82                                               |
| XXXIX   | 3-amy1-7-phenyl-8'-methoxy#        |                                                  |
| XL      | 5,6'-dichloro-8'-methoxy           | 149-152                                          |
| XLI     | 5,8'-dimethoxy-chloro              | 155-157                                          |
| XLII    | 7,8-dimethoxy-6'-chloro            | 104-106                                          |
| XLIII   | 4,7,8'-trimethoxy                  | 104-106                                          |
| XLIV    | 4,7,8'-trimethoxy-6'-chloro        | 126-127                                          |
| XLV     | 6'-nitro-8'-methoxy                | 166-168                                          |
| XLVI    | 6'-methoxy-8'-nitro                | 116-117                                          |
| XLVII   | 4,6,8'-tri methoxy                 | 132-133                                          |
| XLVIII  | 5'-chloro-8'-ethoxy                | 126-127                                          |
| XLIX    | 4,7,6-trichloro-8'-methoxy         | 121-127                                          |
| L       | 5,8'-dimethoxy-6'-bromo            | 125                                              |
| LI      | 5'-bromo-8'-methoxy                | 183-185                                          |
| LII     | 5'-chloro-8'-methoxy               | 160-161                                          |

Those compounds marked \* are most easily transferred in the colored state to another sheet, and those marked # are difficult to transfer in the colored state.

NOTE.—The absence of Roman numerals XVIII and XXVIII in Table I, an otherwise consecutive list, is of no significance.

The preferred compounds, as well as other indolinobenzospiropyran compounds, are made by previously disclosed methods; for example, the method disclosed in The Journal of the American Chemical Society, volume 81, 5605 (1959), which discloses that the general method for making this class of compounds consists essentially of condensing equimolar amounts of a salicylaldehyde compound and a 2-methylene-1,3,3-trimethylindoline compound, both materials being so selected as to provide the desired substituent groups at desired positions on the

condensation reaction products; the methods disclosed in United States Patents Nos. 2,953,454 and 3,100,778; the conventional methods disclosed in Wizinger and Wenning, *Helvetica Chimica Acta*, volume 23, 247 (1940); and methods which are obvious modifications over those cited above and which differ thereover primarily in the use of specific condensation reactants which yield desired indolinobenzospiropyran compounds with the desired substituent group orientation; i.e., at desired ring positions.

The following examples are set forth merely to illustrate the preparative technique for making compounds of the class disclosed above. For this purpose, the details of preparing certain specified compounds of this class appear directly below:

#### EXAMPLE I

##### *The 6'-chloro-8'-methoxy-1,3,3-trimethyl derivative*

A solution of one mole of 3-methoxysalicylaldehyde (Tiemann, Koppe, Ber. 14, 2021 (1881) in 700 milliliters of glacial acetic acid is bubbled with chlorine, the temperature of the solution being held below 20 degrees centigrade, until a yellow precipitate separates. The precipitate is recrystallized from ethanol to give 0.40 mole of 5-chloro-3-methoxysalicylaldehyde with a melting point of 117 to 118 degrees centigrade.

To 0.4 mole of 1,3,3-trimethyl-2-methyleneindolino in 100 milliliters of ethanol is added 0.4 mole of 5-chloro-3-methoxysalicylaldehyde. The mixture is refluxed for two hours, filtered hot, cooled, and filtered again to give 0.35 mole of white powder with a melting point of 125 to 126 degrees centigrade.

This is the preferred chromogenic material for use in practicing the invention.

#### EXAMPLE II

##### *The 4,7,8'-trimethoxy-1,3,3-trimethyl derivative*

One mole of 2,5-dimethoxyaniline, one mole of acetoin, and four moles of zinc chloride are placed in a two-liter flask and heated to 160 degrees centigrade for one hour. The reaction mixture is cooled, washed several times with water, and extracted with ether. The ether is evaporated off and distilled at 153 degrees centigrade/0.8 mm. of Hg to give 0.85 mole of 2,3-dimethyl-4,7-dimethoxyindole.

The indole (0.85 mole) thus obtained is methylated by being heated at 120 degrees for five hours in 100 milliliters of methanol with 2.55 moles of methyl iodide in a two-liter autoclave. The solid thus obtained is washed with

acetone, decomposed with base, extracted with ether, and distilled at 142 degrees centigrade/1.5-2.0 mm. of Hg to give 0.4 mole of 4,7-dimethoxy-1,3,3-trimethyl-2-methyleneindoline.

To one mole of 4,7-dimethoxy-1,3,3-trimethyl-2-methyleneindoline in 200 milliliters of ethanol is added one mole of 3-methoxysalicylaldehyde (Tiemann, Koppe, Ber. 14, 2021 (1881)). The mixture is refluxed for two hours, filtered while hot, cooled, and filtered a second time. The precipitate is recrystallized from ethanol to give 0.93 mole of white powder, melting point 105 to 106 degrees centigrade.

#### EXAMPLE III

##### *The 5-chloro-8'-methoxy-1,3,3-trimethyl derivative*

To one mole of 5-chloro-1,3,3-trimethyl-2-methyleneindoline (Soc. Anon. Pour l'Ind. Chim. A Bale, Heinrich von Diesbach, Swiss 137,943, May 19, 1928) in 200 milliliters of ethanol is added one mole of 3-methoxysalicylaldehyde (Tiemann, Koppe, Ber. 14, 2021 (1881)). The mixture is refluxed for two hours, filtered hot, cooled and filtered a second time. The precipitate is recrystallized from ethanol to give 0.90 mole of white crystals, melting point 140 to 141 degrees centigrade.

#### EXAMPLE IV

##### *The 1-phenyl-8'-methoxy-3,3-dimethyl derivative*

To one mole of 1-phenyl-3,3-dimethyl-2-methyleneindoline (Brunner, Ber. 31, 1943 (1898)) in 200 milliliters of ethanol is added one mole of 3-methoxysalicylaldehyde (Tiemann, Koppe, Ber. 14 2021 (1881)). The mixture is refluxed for two hours, filtered hot, cooled, and filtered a second time. The precipitate is recrystallized from ethanol to give 0.90 mole of white crystals, melting point 163 to 164 degrees centigrade.

#### EXAMPLE V

##### *The 8'-ethoxy-1,3,3-trimethyl derivative*

To one mole of 1,3,3-trimethyl-2-methyleneindoline (Brunner, Ber. 31, 1943 (1898)) in 200 milliliters of ethanol is added one mole of 3-ethoxysalicylaldehyde (Davies, J. Chem. Soc. 123, 1587 (1923)). The mixture is refluxed for two hours, filtered hot, cooled, and filtered a second time. The precipitate is recrystallized from ethanol to give 0.85 mole of white crystals, melting point 83 to 85 degrees centigrade.

#### The phenol compounds

| Structure | Formula                       | M.P., °C. |
|-----------|-------------------------------|-----------|
| A.....    | 4-tertiary butylphenol.....   | 94-99     |
| B.....    | 4-phenylphenol.....           | 166-167   |
| C.....    | 4-hydroxydiphenyloxyde.....   | 85        |
| D.....    | α-Naphthol.....               | 95-96     |
| E.....    | β-Naphthol.....               | 119-122   |
| F.....    | Methyl-4-Hydroxybenzoate..... | 126-128   |
| G.....    | 4'-hydroxyacetophenone.....   | 108-110   |

| Structure                                                                           | Formula                                             | M.P., °C. |
|-------------------------------------------------------------------------------------|-----------------------------------------------------|-----------|
|    | 4-tertiary-Octylcatechol                            | 109       |
|    | 2,2'-dihydroxydiphenyl                              | 103-109   |
|    | 2,2'-methylene bis(4-chlorophenol)                  | 164       |
|    | 2,2'-methylene bis(4-methyl-6-tertiary butylphenol) | 125-130   |
|    | 4,4'-isopropylidenediphenol                         | 156       |
|    | 4,4'-isopropylidene bis(2-chlorophenol)             | 90-91     |
|   | 4,4'-isopropylidene bis(2,6-dibromophenol)          | 172-174   |
|  | 4,4'-isopropylidene bis(2,6-dichlorophenol)         | -----     |
|  | 4,4'-isopropylidene bis(2-methylphenol)             | 136       |
|  | 4,4'-isopropylidene bis(2,6-dimethylphenol)         | 108       |
|  | 4,4'-isopropylidene bis(2-tertiary butylphenol)     | 109-114   |
|  | 4,4'-sec. butylidenediphenol                        | 118-121   |
|  | 4,4'-sec. butylidene bis(2-methylphenol)            | 142       |
|  | 4,4'-cyclohexylidenediphenol                        | 180       |

| Structure                                                                         | Formula                                     | M.P., ° C. |
|-----------------------------------------------------------------------------------|---------------------------------------------|------------|
|  | 4,4'-cyclohexylidene bis (2-methyl-phenol). | 184        |
|  | 2,2'-thio bis (4,6-dichlorophenol)          |            |

## The Color combinations

Following is a representative group of pairs of the color reactants and the color produced by their reaction.

| Chromogenic material | Phenol material | Color              |
|----------------------|-----------------|--------------------|
| I                    | A               | Blue-black.        |
| I                    | B               | Do.                |
| I                    | C               | Purple-black.      |
| XL                   | C               | Green-blue.        |
| VI                   | C               | Green.             |
| XLIII                | C               | Purple-black.      |
| I                    | D               | Brown-black.       |
| XL                   | D               | Blue-green.        |
| XLIII                | D               | Brown.             |
| VI                   | D               | Dark green.        |
| XLIII                | D               | Brown.             |
| I                    | E               | Brown-black.       |
| I                    | F               | Green-brown.       |
| XL                   | F               | Green.             |
| VI                   | F               | Light green.       |
| XLIII                | F               | Brown.             |
| I                    | G               | Green-brown.       |
| XL                   | G               | Green.             |
| VI                   | G               | Do.                |
| XLIII                | G               | Brown.             |
| I                    | H               | Dark purple.       |
| XL                   | H               | Blue-black.        |
| VI                   | H               | Brown-green.       |
| XLIII                | H               | Dark purple.       |
| I                    | I               | Dark brown.        |
| XL                   | I               | Brown.             |
| VI                   | I               | Green-brown.       |
| XLIII                | I               | Brown.             |
| I                    | J               | Do.                |
| XL                   | J               | Green-brown.       |
| VI                   | J               | Brown.             |
| XLIII                | J               | Do.                |
| I                    | K               | Green-gray.        |
| XL                   | K               | Light gray.        |
| XLIII                | K               | Green-gray.        |
| I                    | L               | Blue-black.        |
| XXV                  | L               | Dark blue.         |
| XL                   | L               | Green-blue.        |
| VI                   | L               | Green.             |
| XLIII                | L               | Purple-black.      |
| I                    | M               | Dark brown.        |
| XXV                  | M               | Blue-black.        |
| XL                   | M               | Blue-gray.         |
| VI                   | M               | Light gray.        |
| XLIII                | M               | Dark brown.        |
| I                    | N               | Light gray.        |
| XL                   | N               | Do.                |
| XLIII                | N               | Do.                |
| I                    | O               | Light gray/yellow. |
| XXV                  | O               | Gray blue.         |
| XL                   | O               | Light gray.        |
| XLIII                | O               | Brown.             |
| XXV                  | P               | Dark blue.         |
| XXV                  | Q               | Light blue.        |
| I                    | R               | Green-blue.        |
| XXV                  | R               | Blue.              |
| XL                   | R               | Light green/blue.  |
| VI                   | R               | Light gray.        |
| XLIII                | R               | Green-blue.        |
| I                    | S               | Purple-black.      |
| XXV                  | S               | Blue-black.        |
| XL                   | S               | Blue-gray.         |
| VI                   | S               | Green.             |
| XLIII                | S               | Purple-black.      |
| XXV                  | T               | Dark blue.         |
| XXV                  | U               | Green-black.       |
| I                    | V               | Blue.              |
| XXV                  | V               | Brown.             |
| XL                   | W               | Light brown.       |
| VI                   | W               | Orange.            |
| XLIII                | W               | Brown.             |

As to the organization of materials in functional arrangement

The particles of sensitizing materials in unreacted colorless state or in reacted colored state may be organized

with respect to support material and with respect to mark-receiving material in a number of ways to make possible 20 the production of multiple copies at once or serially, or to make recordings, on a single sheet or by use of a master sheet.

The preferred support sheet is paper because of its durability, absorbence, light and heat coefficients, opaqueness or translucence as desired, cheapness, and flexibility. 25 However, film sheets of polymeric material, woven sheets, or bands of laminated materials may be used. The sheet used may be impregnated or coated with the sensitizing materials, such coating or impregnation fitting the proposed use as to depth of penetration of the reactants if penetration is involved, or with respect to the location of the reactants as to the broad surfaces of the sheet, or with respect to amounts and kinds of reactants. If the sheet is of solid film material, it should be penetrable 30 by the fluid state of the reactants, or else the sensitizing materials should be situated at or on the surface of the sheet. The support material can be the surface of a thick plate, or of other more substantial structure than the sheet or plate form, providing that the support material does not 35 act as a heat-sink to any large degree so that it interferes with the production of temperatures necessary to make marks or to transfer marks or marking reactants. The sheets should be as thin as is consistent with the proposed use, and for some purposes may be opaque and for other purposes may be of a translucent character, to 40 enable data recorded on one side to be read from the other side. For the purposes of this disclosure, unless otherwise specified, it is to be considered that the support sheet is thin, relatively opaque white paper, and that any 45 written or printed data to be used in conjunction therewith for control of recording be of a marking material that is 50 raised in temperature relatively to the supporting member when both are commonly irradiated by infra-red radiation.

The particles of phenol material should be as small in size as is consistent for the necessary resolution and coating properties—such as, say, around three microns in average largest dimension—and the particles of chromogenic material should be of similar dimensions, although the size is not critical if the optical effect is sufficiently 55 good with respect to resolution, as may result from the materials having been in mobile condition. In respect to resolution, the particles preferably should be supplied in such quantity in an area to be served as to give no perception of individual existence. All of the named materials 60 either are colorless (white in powdered form) or have such small coloration in the unreacted form that they may be considered as leuco compounds.

Where no binder is to be used, it is important that the two reactants in unreacted state be on different sheets, insulated by space or an intermediate insulator means until just before use, and separated thereafter if any unreacted materials remain in contact. Either reactant can exist alone on a sheet, or the reactants in reacted colored state can exist together with an unreacted residue, with

out physical insulation, and even one of the reactants can exist on a sheet in the presence of the reaction product mark without desensitizing the unreacted remaining area. Ordinarily, if two reactants are to be stored unreacted on the same sheet, they are disposed on the sheet with about a maximum of 25% or 30% of binder material to leave a thin film of such material around each of the particles that will not obstruct passage of the reactants in mobile condition in a recording operation. To further protect such a sheet from rough handling, or winding or stacking pressures, an overcoating of some film material is applied. It is within the scope of the invention to have the unreacted materials alone or in combination in a data-representing configuration or pattern on a sheet, such a pattern acting to control the transfer of material in the form of a pattern to an under sheet by a hot member applied generally to the sheet as distinguished from the application of heat in a pattern as determined by hot type or by thermography procedures.

Where both reactants are on the same sheet, they may be in interspersion or in layers, be one or both on the surface, partly beneath the surface, or entirely beneath the surface of a sheet. If in layers, the reactants with binder materials will not obscure vision of recorded data, as, at points where marks are produced, a fusion of the superimposed materials occurs.

It is within the scope of the invention, and is, indeed, an important part of the invention, to provide for the making of a master sheet copy from which a number of second-generation copies of a document may be made onto plain paper by heat and contact, without regard for or requiring the presence of the original document, or even as an incident of use of the original document if its back is sensitized according to one aspect of this invention.

The structural combination of elements in a number of forms illustrative of the invention is shown in the drawings which form part of this specification but which are not to be deemed to limit the claimed subject matter.

#### Of the drawings:

FIG. 1 is a schematic diagram of several constructions in cross-section of a sheet supplied with the reacting compound particles, (a) showing a sheet of film material or paper having the reactant particles located on a surface in interspersion, (b) showing the color reactant buried throughout a sheet of paper and the phenol reactant on a surface, (c) showing the reverse of (b), and (d) showing both reactants buried in interspersion in a paper sheet;

FIG. 2 is a schematic showing in (a) two facing record sheet surfaces, the facing surfaces being sensitized with the co-reactants, and showing how infra-red radiation is used in conjunction with a "thermographic" ink print to make a mark, view (a) showing two sheets stapled as a unit, and view (b) showing a folded sheet with a severance formation served with an interleaf sheet carrying one of the reactants. In FIG. 2, it is assumed that the chromogenic material is not rendered mobile by the temperatures used, but the phenol is transferred;

FIG. 3 shows both reactants on the rear surface of a sheet bearing thermographically-responsive data on the front surface, so that heat engendered by infra-red radiation striking the data heats it, which heat turns the materials on the rear surface to a pattern of colored mobile fluid which is transferred to a plain sheet of paper placed in contact therewith; and

FIG. 4 shows an overlying sheet of paper having a mirror-image of data recorded in terms of one or both of the reactants on the rear surface of a sheet, so that it may be passed to a plain sheet in a mobile fluid phase by a heat press; the plain sheet also may be supplied with one of the necessary reactants if it is missing, by intention, from the overlying sheet.

Preliminary to specifying how the record member sheets are made, it should be understood that, if the reactant material is to be applied to a base sheet as a solution, it should not come into contact in the liquid solution state

with the other reactant, because color will be produced prematurely. In those instances where a sheet is to be entirely coated with the reaction product, for transfer purposes, the reactants may be applied as solutions and dried. However, for all the purposes of this invention, the preferred form of applying the reactant materials is by coating a non-solvent liquid dispersion thereof on the base sheet.

In the event that reactant surfaces of two sheets are to be placed or kept in contact, or a stack of sheets having the two reactants coated on one side is to be kept in storage, either as already-made records or as sheets to be recorded upon, a protective overcoating of film material of one to two pounds per ream of 25-inch by 38-inch sheets is applied to the active surfaces. As an effective example of such protective coating composition, the following is specified:

#### Protective overcoating.—Composition

|                               | Parts by weight |
|-------------------------------|-----------------|
| Polyvinyl alcohol             | 75              |
| Sodium carboxymethylcellulose | 25              |
| Water                         | 1,000           |

In the following discussion of the preparation and use of different kinds of coated sheets, sheets I, II and III are those illustrated in the drawings. In each case the sheets so designated may have a light coating weight (sheets IA, IIA, and IIIA) for use as receiving or copy sheets or a heavier coating weight (sheets IB, IIB and IIIB) for use as transfer sheets. In the discussion, "sheet I," "sheet II," or "sheet III" is used to designate the sheets in cases where it is not necessary or appropriate to designate the coating weight. The A and B designations are added where the coating weight of the sheet is relevant to the discussion.

#### Making a phenol-particle-coated sheet I

A ball mill is loaded with the following composition:

|                                             | Parts by weight |        |
|---------------------------------------------|-----------------|--------|
|                                             | Wet             | Solids |
| 4,4'-isopropylidene di-phenol               | 85              | 85     |
| Water                                       | 115             | 200    |
| Hydroxyethylcellulose 7.5% aqueous solution | 15              | 15     |

and the contents milled until the average particle size of three microns is reached. For use as a receiving sheet of this construction (sheet IA), a base paper sheet should be coated to provide a dried weight of one to two pounds per ream as specified. Any desired base paper stock sheet is useful. Where the di-phenol portion of the coated material is to be transferred to another sheet, the coating composition should be used in an amount to yield a four-to-five-pound dried weight per ream, which sheet with this weight of coating is referred to as sheet IB.

#### Making a sheet coated with chromogenic particles.—Sheet II

A ball mill is loaded with the following composition:

|                                                                | Parts by weight |     |
|----------------------------------------------------------------|-----------------|-----|
|                                                                | Wet             | Dry |
| 1,3,3-trimethyl-6'-chloro-8'-methoxy-indolino-benzo-spiropyran | 70              | 70  |
| Polyvinyl alcohol (88% hydrolyzed) 7.5% solution in water      | 400             | 30  |
| Water                                                          | 30              | 30  |

and the contents milled to an average particle size of three microns. For use as a receiving sheet (sheet II A), a one-to-two-pound, dried weight, coating per ream, as specified, is sufficient, whereas for a transfer sheet of this construction (sheet II B), three to four pounds dried weight per ream should be used.

Making a sheet coated with both phenol particles and chromogenic particles III

A ball mill is loaded with the following composition:

|                                                                    | Parts by weight |       |
|--------------------------------------------------------------------|-----------------|-------|
|                                                                    | Wet             | Dry   |
| 4,4'-isopropylidene di-phenol.....                                 | 70              | 70    |
| 1,3,3-trimethyl-6'-chloro-8'-methoxy indolino-benzospiropyran..... | 15              | 15    |
| Hydroxyethylcellulose (low viscosity) 7.5% solution in water.....  | 200             | 15    |
| Water.....                                                         | 115             | ..... |

and is run until the solid particle size averages three microns, to form a coating material which is applied to paper in an amount to yield a coating of two to three pounds per ream, dried weight, for use as a heat-responsive copy sheet (sheet III A). If a reflex copy system is used—that is, where the sheet must be penetrated by infra-red light—a thin paper base sheet is used. For use as a transfer sheet (sheet III B), three to five pounds, dried weight, of coating per ream is used.

A protective overcoating should be used with these sheets when they are in close storage.

Equivalent binder materials

Equivalents for hydroxyethylcellulose as binder materials are:

methylcellulose  
gum arabic \*  
gelatin  
casein \*  
zinc caseinate \*  
sodium carboxymethylcellulose  
polyvinyl alcohol  
pectin  
polyvinylpyrrolidone  
starch and starch derivatives  
styrene maleic anhydride copolymers \*  
polyethylene-maleic anhydride copolymers  
polyvinylpyrrolidone-maleic anhydride copolymers  
polyacrylates and copolymers of them  
latices of butadiene-styrene;  
vinyl chloride; acrylic,  
vinyl acetate, etc.,

those followed by an asterisk being found most useful.

The use of Sheets I and II together

In this instance of use, sheets I and II (FIG. 2a) are placed in face-to-face relation, and either can be the copy sheet. The original data is pre-recorded on the uncoated side of the selected sheet to provide thermographic responsive representation of the data. On heating of the data with infra-red radiation, while the coated sides are in contact, the copy will appear on the coated surface of both sheets. The infra-red radiation, in the interests of efficiency, should be applied directly to the thermographically responsive data. It is thus to be noted that either sheet I or sheet II can be a copy-receiving sheet; in this instance,

sheet II has a mirror-image of the data. If the copy made is to be transferred, then the heavier coatings should be used, typified by specified sheets IA and II A. Direct reading images and mirror-images, therefore, may be made according to the arrangement of sheets with respect to each other, and the applied energy, according to the well-known optical and transfer laws governing copying procedures.

The use of sheet III

10 This sheet III may be used alone as a copy-receiving sheet by being served with a pattern of heat from front or back, as by thermographic original document, by trace of a hot stylus, by hot type, or by any other means giving 15 a differential heat pattern.

If the heavier coating is used, the sheet may be used for a transfer sheet to produce multiple copies on plain surfaces of any sort, such as bond paper, newsprint, cloth, film, and the like, as long as the pattern of heat is present to control the transfer.

The use of an interleaved sheet

If the document to be copied is not sensitized on the 25 rear surface, the missing reactant may be supplied by means of an interleaved sheet, as shown in FIG. 2b.

The use of sheet III as a master sheet (direct)

30 Sheet III, as the more heavily coated sheet (sheet II B), has the data to be recorded printed on the uncoated side. The coated side is placed against plain paper to form a record "pair," which is passed by a light source of infra-red wave length, so that the radiation directly strikes the 35 printing. A copy of the recorded data will appear on the plain paper. This can be repeated until the coating is exhausted.

The use of sheet III (or sheets I and II) as a master sheet (intermediate)

The heavier coated sheet II B is written on with thermographic ink directly on the coated side. A piece of plain paper is placed in contact with the writing on 45 sheet II B to form a pair, and the pair is subjected to infra-red radiation. This puts a colored mirror-image of the recorded data on the plain paper. This plain sheet then may be used over and over against successive sheets of plain paper, and each pair is subjected to a hot press 50 to transfer the colored image in direct reading form.

If a sheet II A has recording on its coated side in terms of thermographic ink, and a pair is formed by contact of a plain sheet of paper placed thereagainst and subjected to infra-red radiation, the mirror-image of the 55 recorded data will appear on the plain sheet in mirror-image form. This mirror-image then is transferred to the coated surface of a sheet II and subjected to application of heat by use of a hot plate. The direct reading image will appear on sheet II, and this operation may be repeated 60 with other type II sheets until the pattern of material is exhausted.

If a sheet II A has a recording on its coated surface in terms of thermographic ink and is pressed against a sheet I type coated surface and the pair is subjected to infra-red radiation, it forms a mirror-image master sheet, which 65 may be used to transfer the data to a type I sheet successively until the mirror-image is exhausted.

It has been mentioned that the reactant materials in whole, or in part, may be placed within the boundaries 70 of a sheet, and such placement may be made by mixing particles of the reactant in the head-box furnish of a paper-making machine, or coated on a wet sheet of paper-stock furnish before the drying of it to a completed paper sheet. The amount and the depth of distribution of the 75 buried particles all have a bearing on the effectiveness

of such sheets, and optimum conditions quantitatively can be determined for a particular base sheet, energy source, and other variable factors by empirical test, all well within the skill of one familiar with the art.

While many phenol compounds, particularly di-phenol compounds, have been disclosed, it is their acidic nature in the mobile fluid state of the material that makes them valuable for carrying out and practicing the invention; hence equivalents in acid activity and in ability to form a mobile fluid phase at thermographic temperatures, together with low vapor pressure at temperatures below 60 degree centigrade, are to be considered as forming a criterion for the selection of equivalents.

What is claimed is:

1. A record member including a support sheet having a record surface of solid particles of phenol material as a first reactant and solid particles of chromogenic benzo-indolinospiropyran material as a second reactant which is colorable on reaction contact with the phenol material, said particles of phenol and chromogenic material reactants producing color by at least one of the reactants becoming mobile as a fluid phase at temperatures associated with thermographic phenomena, said solid phenol particles being insulated from solid contact with the proximate solid particles of chromogenic material by a thin polymeric material film that is pervious to the thermographically-produced mobile phases of the reactant materials.

2. The record material of claim 1 in which the phenol material is of the di-phenol class.

3. A record member including a support sheet having a record surface of minute particles of phenol material which are solid at the maximum living environment temperature (60 degrees centigrade) and having a mobile fluid phase in marking quantity at the higher temperatures encountered in thermographic phenomena, and proximately positioned in contiguity to, but spaced apart from, the particles of phenol by a polymeric material film, an equivalent, from a reaction standpoint, amount of solid particles of chromogenic material of the benzo-indolinospiropyran type also being solid at temperatures below 60 degrees centigrade and having a mobile fluid phase at temperatures associated with thermographic phenomena, said polymeric material affording isolation of the solid particles of chromogenic material from the solid particles of phenol but passing either kind of particles material in the mobile fluid state phase produced by thermographic temperatures.

4. A sheet of record material having on a surface thereof a visually continuous coating of the reaction product of a di-phenol compound and a benzo-indolinospiropyran compound, said reaction product being convertible to a mobile fluid phase by temperatures associated with thermography.

5. A sheet of record material having on a surface thereof a heat-transferable coating of the reaction product of a di-phenol compound and a benzo-indolinospiropyran compound arranged in data-representing configuration.

6. A sheet of record material having on a surface thereof a heat-transferable coating of the reaction product of a phenol compound and a benzo-indolinospiropyran compound.

7. The record material of claim 6 wherein the coating is arranged in the configuration of recorded data, whereby a general heating of the record material will produce a mobile fluid phase of the recorded data as a colored pattern for transfer to another sheet by contact.

8. The sheet of record material of claim 6 in which the benzo-indolinospiropyran compound is the compound



5

10

15

20

25

30

35

40

45

50

55

55

60

65

9. A sheet of record material having on a surface thereof a coating of the reaction product of a phenol compound and a benzo-indolinospiropyran compound arranged in data-representing configuration.

10. A method of making copies of recorded data on plain paper including the steps of forming on a surface of a proposed master sheet the mirror-image of the data in terms of the reaction product of a phenol compound and a benzo-indolinospiropyran compound; placing the mirror-image surface against a plain paper sheet to form a contact pair; and applying heat to the pair sufficient to form a mobile fluid phase of the reaction product image and to transfer such a portion of said fluid phase to the plain paper as adheres thereto.

11. A pair of record material sheets operable in face-to-face contact, each sheet being supplied with material in solid form which turns to a mobile fluid phase at temperatures associated with thermographic phenomena and the material on one sheet reacting on contact with the material on the other sheet, if only one of the materials is in a fluid state, to produce a distinctive color, one of the component materials being a phenol compound and the other material being a chromogenic benzo-indolinospiropyran compound, both materials being in solid state below 60 degrees centigrade.

12. A master sheet for use in controlling and supplying material for the production of multiple copies of data on successively presented sheets of copy record material brought into contact therewith, said master sheet having on the contacting surface a transfer coating including a finely interspersed juxtaposed array of particles including a phenol compound and a benzo-indolinospiropyran compound which react at thermographic temperatures to produce a marking material capable of transfer to a copy-receiving sheet.

#### References Cited

##### UNITED STATES PATENTS

- |           |         |                    |             |
|-----------|---------|--------------------|-------------|
| 2,967,785 | 1/1961  | Allen et al. ----- | 117—36.8 XR |
| 3,239,366 | 3/1966  | Miller et al.      |             |
| 3,244,550 | 4/1966  | Farnham et al. --- | 101—473 XR  |
| 3,262,386 | 7/1966  | Gordon -----       | 101—469     |
| 3,280,735 | 10/1966 | Clark et al. ----- | 101—470     |

DAVID KLEIN, Primary Examiner.

U.S. Cl. X.R.

96—90; 101—470, 473; 117—36.2, 36.7, 36.8, 36.9; 250—65